

# UNITED STATES PATENT OFFICE.

CONRAD PAUL HUBERT CLAESSEN, OF WILMERSDORF, NEAR BERLIN, GERMANY.

## SMOKELESS GUNPOWDER.

No. 909,546.

Specification of Letters Patent.

Patented Jan. 12, 1909.

Application filed August 9, 1906. Serial No. 329,801.

*To all whom it may concern:*

Be it known that I, CONRAD PAUL HUBERT CLAESSEN, doctor of philosophy, chemist, subject of Prussia, residing at Wilmersdorf, 5 near Berlin, Germany, have invented new and useful Improvements in Smokeless Gunpowder, of which the following is a specification.

In order to lower the temperature of combustion of the nitrocellulose powders or of the nitrocellulose-nitroglycerin powders, and in order to remove the injurious influence which said temperatures exert upon the material of the barrel or the tube, indifferent 15 substances, for example camphor, were hitherto added to powders of this kind and, in order to increase the stability, diphenylamin or carbamids were also used as addition to these powders.

Now it has been proved by experiments 20 that the above named purposes, that is the lowering of the temperature of combustion and the increase of the stability of such powders are attained in a much higher degree, without injuring, at the same time, the ballistic properties of the powders, if there are 25 added to the latter entirely substituted carbamids, that is to say, such carbamids in

which the four hydrogen-atoms of the ammonia rests are replaced by organic radicals. 30 For instance the diethyl-diphenyl-carbamid has proved to be excellently adapted for the above named purposes. Besides, these tetra-substituted carbamids have also the advantage over those substances that have hitherto 35 been used, that they are not volatile, as is the case, for instance, with camphor.

A nitrocellulose powder according to my invention may consist of 100 kg. of gun cotton, 5 kg. of diethyldiphenylcarbamid. 40

A nitrocellulose nitroglycerin powder according to my invention may consist of 75 kg. of gun cotton, 25 kg. of nitroglycerin, 5 kg. of diethyldiphenylcarbamid. 45

I claim:—

A smokeless gunpowder consisting of a mixture of nitrocellulose and nitroglycerin with about 5% diethyl-diphenyl-carbamid.

In testimony whereof I have signed my name to this specification in the presence of 50 two subscribing witnesses.

CONRAD PAUL HUBERT CLAESSEN.

Witnesses:

HENRY HASPER,  
WILLIAM MAYNER.